

## UNITED STATES PATENT OFFICE

2,067,929

## PROCESS OF DYEING WITH VAT DYES

Jean G. Kern, Hamburg, N. Y., assignor to National Aniline & Chemical Company, Inc., New York, N. Y., a corporation of New York

No Drawing. Application April 8, 1935, Serial No. 15,262. In Japan September 3, 1934

9 Claims. (Cl. 8—5)

This invention relates to the art of dyeing with vat dyes. It relates especially to a new class of assistants for the dyeing of textile fibers, and especially those of the vegetable type, such as cotton, regenerated cellulose and the like, with vat dyes by means of a dye bath or dye liquor containing a vat dye in the reduced form, whereby dyeings of excellent fastness, penetration, depth and brilliance may be obtained.

As is well known, vat dyes are solid substances which are insoluble in water. In the dyeing of textile fibers with vat dyes, the insoluble vat dyes are converted to a reduced form, in which form they are taken up by the fiber, and then the fiber is subjected to an oxidizing or fixing treatment whereby the dyestuff is again rendered insoluble. In general, the dyeing process involves treatment of the fiber to be dyed with the dye bath or dye liquor, containing the reduced compound (leuco-compound) of the vat dye. A number of procedures are employed in carrying out the process, as for example, working piece goods (cotton, regenerated cellulose, etc.) and raw cotton stock (unspun cotton fiber) in the dye bath (vat), pad dyeing piece goods by passing rapidly through the dye bath, treating raw cotton stock in a dyeing machine with the dye liquor, working yarn on beams in the dye bath, treating yarn in package dyeing machines with the dye liquor, etc.

The preparation of the dye bath or dye liquor generally involves diluting with water a vat dye paste or powder (containing the vat dye in the ordinary, unreduced form, usually after screening to insure desired fineness of the vat dye particles) and mixing it with alkali (e. g. sodium hydroxide) and a reducing agent (e. g. sodium hydrosulfite) in suitable amounts to form a bath of the reduced (leuco) compound of the vat dye, while heating to the temperature suitable for the particular vat dye used. The resulting bath or liquor is then employed in the dyeing operation.

For economical dyeing it is desirable that maximum utilization of the vat dye be secured, that the dyeings be thoroughly penetrated, and that the color be uniform (level) and bright.

The present invention is based upon the discovery that the soluble salts of the acid reaction products resulting from the interaction of an aliphatic alcohol containing less than 6 carbon atoms with a polybasic inorganic acid or suitable derivative thereof possess a combination of properties which render them of particular value for use as assistants in the dyeing of textile fibers, and especially those of the vegetable type, such as cotton, rayon (regenerated cellulose) and the

like, by a process in which the fiber to be dyed is treated with a non-acid dye bath or dye liquor containing a vat dye in the reduced (leuco) form and preferably also containing an alkali. Thus, the soluble salts of the acid reaction products of sulfuric acid or chlorosulfonic acid upon the aliphatic monohydric alcohols which contain 5 or less carbon atoms, which products are considered to be acid alkyl sulfates corresponding with the formula  $ROSO_3H$  (in which R is a hydrocarbon radical containing not more than 5 carbon atoms), as well as others of the hereinafter described soluble salts of acid alkyl esters of inorganic polybasic acids, have no tendency to cause the resulting dye baths and dye liquors to foam or lather by reason of the presence of the said salts. They have the further advantageous property of acting as assistants in the absorption or adsorption of the reduced compounds of the vat dyes by the fiber, and in the penetration of woven fabric by the reduced compounds of the vat dyes. The alkyl ester salts of the present invention apparently act on both the vat dye and the fiber itself, causing more effective absorption of the leuco compound of the dye.

The acid alkyl esters, the soluble salt of which may be employed in accordance with the present invention, include the partial esters of polybasic inorganic acids (as for example, of sulfuric, phosphoric, boro-sulfuric, boro-phosphoric, boric, silicic, etc., acids) and especially those of sulfuric and phosphoric acids, containing at least one aliphatic hydrocarbon radical (straight-chain, branched-chain, saturated or unsaturated) which contains not more than 5 carbon atoms, as the organic (ester) radical or radicals. These partial esters (which are herein designated as "acid alkyl esters") may be represented by the formula  $(RO)_x-A-(OH)_{n-x}$

in which

R represents an aliphatic hydrocarbon radical which contains not more than 5 carbon atoms,

A represents the residue of the inorganic acid (as for example, the radical  $SO_2$ , the radical  $PO$ , the radical  $SiO$ , the radical B, etc.),

n represents the number of hydrogen atoms, in the uncombined polybasic acid from which the ester is derivable which are replaceable by a metal (herein designated as "replaceable hydrogen atoms"), and x is 1 or more but not greater than n—1.

As is well known a partial ester, or acid alkyl ester, of a polybasic inorganic acid is an ester in which at least one of the replaceable hydrogen

atoms of the parent polybasic inorganic acid has not been replaced.

It is to be noted, in the case of acid alkyl esters which are derivatives of polybasic acids containing 3 or more replaceable hydrogen atoms in which more than one of said hydrogen atoms has been replaced by organic radicals, the said organic radicals (represented by R in the above formula) may be the same or different.

10 The alkyl ester salts employed in accordance with the present invention comprise especially the soluble salts of the herein described acid alkyl esters, e. g., those resulting from the combination of any suitable metal or base, including the organic bases, with the said acid alkyl esters. It is particularly advantageous, however, to use the alkali metal salts of the acid alkyl sulfates, phosphates, boro-sulfates and boro-phosphates or the salts formed by the interaction of the said alkyl sulfates, phosphates, boro-sulfates and boro-phosphates with aliphatic or aromatic amines, for example, the alkylol amines. Thus the potassium and sodium salts of the said acid alkyl esters, or the salts of the acid alkyl esters with diethanolamine, triethanolamine, pyridine, or other salt-forming ammonium bases, may be used. The sodium salts, in view of their extremely high solubility in water and alkaline dye baths and dye liquors are of especial value.

15 30 The said salts of alkyl esters employed in accordance with the present invention may be prepared in any manner well known to the art; as for example, by the treatment of the corresponding alcohol, in the presence or absence of a solvent or diluent, with a suitable inorganic reagent (such as phosphoric acid, phosphorus chloride or oxy-chloride, concentrated sulfuric acid, and/or chlor-sulfonic acid, and/or one or more of these in the presence of boric acid, etc.) and neutralization 35 of the resulting acid alkyl ester with an inorganic or organic base which forms a readily soluble salt with said acid alkyl ester. It may be noted that the alkyl sulfuric acids and the alkyl boro-sulfuric acids resulting from the use of sulfuric acid or 40 chlorosulfonic acid, in the absence or presence of boric acid, may contain varying amounts of sulfonic acids which are sometimes produced due to secondary reactions; the presence of such sulfonic acids, however, does not impair the usefulness 45 of the alkyl sulfuric acids, and alkyl boro-sulfuric acids in accordance with the present invention.

50 As illustrating acid alkyl esters, the soluble salts of which may be employed in accordance with the present invention, the following may be mentioned: the mono-ethyl, propyl, butyl and amyl sulfuric acids; the ethyl, propyl, butyl and amyl boro-sulfuric acids; the mono- and di-ethyl, propyl, butyl and amyl phosphoric acids; the ethyl, propyl, butyl and amyl boro-phosphoric acids, etc.

55 60 Of special interest in connection with the present invention are the various soluble salts, and particularly the alkali metal and organic amine salts, of the sulfuric acid monoesters of the various monohydric alcohols which contain not more than 5 carbon atoms, including those which contain single or multiple bonds, straight chains and branched chains; as for example, the sodium or 65 potassium salts of the following: ethyl sulfuric acid; normal and isopropyl sulfuric acids; the mono-sulfuric acid ester of methyl ethyl carbinol; normal-, iso-, and tertiarybutyl sulfuric acids; the mono-sulfuric acid esters of pentasol, of secondary butyl carbinol, and of methyl-n-propyl

carbinol; pentene-2-sulfuric acid; normal amyl sulfuric acid; tertiary amyl sulfuric acid; amylene sulfuric acid; etc. The salts of the monoalkyl sulfuric acids which contain from 3 to 5 carbon atoms in the alkyl group are of especial value in dyeing with vat dyes in accordance with the present invention. Those in which the alkyl group comprises an iso-alkyl radical (as for example, an isopropyl radical:



10 an isobutyl radical:



15 20 are somewhat superior in their action to those in which the alkyl group is a normal or straight-chain radical.

The said sulfuric acid mono esters may be prepared, for example, by the treatment of the corresponding alcohol, in the presence or absence of a solvent or diluent, with a suitable sulfonating agent (such as concentrated sulfuric acid and/or chlorosulfonic acid or the like), or by the interaction of sulfuric acid or the like with the corresponding unsaturated hydrocarbon. Thus, a suitable alcohol dissolved in an inert organic solvent may be reacted with the necessary amount of sulfonic acid to form the sulfuric acid mono ester of the alcohol, the mixture then may be blown with air to remove hydrogen chloride formed, and subsequently stirred with water.

25 30 Mixtures of salts of the said acid alkyl esters may also be employed in accordance with the present invention. For example the salts of suitable inorganic or organic bases with the commercially available and cheap mixtures of alkyl sulfuric acid resulting from the sulfuric acid treatment of mixed gaseous and lighter liquid unsaturated hydrocarbons, such as the mixtures produced in the recovery and removal of unsaturated hydrocarbons in the production and purification of gasoline in the so-called "cracking" process of petroleum distillation.

35 40 The percentage of assistant of the present invention that may be employed is not critical and improved results are obtained with even as little as 1 per cent or 2 per cent (based on the total weight of the dye bath or dye liquor).

45 50 The advantageous action of the said salts of the acid alkyl esters may be secured in a number of ways. Thus the said alkyl ester salts may be incorporated into the usual dye baths and dye liquors or into the dyestuff pastes employed in preparing the dye baths and dye liquors. The said alkyl ester salts are in general crystalline products and hence may be added directly to the usual dye baths or dye liquors to cause the desired effect. Further, an advantageous action may be secured by subjecting the cloth to be dyed to a preliminary treatment with the solution of the said alkyl ester salt, as for example, impregnation. In copending application Serial No. 673,030, filed May 26, 1933, vat dye compositions in the form of powders are described containing vat dyestuffs and alkyl ester salts of the type herein disclosed. Such compositions, in view of their content of said alkyl ester salts, may be employed in accordance with the present invention merely by substituting them

5

10

15

20

25

30

35

40

45

50

55

60

65

70

75

for the vat dye pastes usually employed and dyeing in the ordinary manner.

The acid alkyl esters may also be employed as such in dye liquors containing alkali inasmuch as the salts of said acid alkyl esters will be formed in the resulting compositions and there exert their advantageous action.

If desired, foam-breaking or foam-preventing agents may also be included in the compositions 10 of the present invention in connection with vat dyes which have a tendency to produce foaming.

The invention may be employed in connection with vat dyes of all types including those derived from anthraquinone, indophenols, various 15 indigoid, thioindigoid and indirubin compounds, etc.; as for example, indanthrones, pyranthrones, flavanthrones, dibenzanthrones, isodibenzanthrones, perylene quinones, anthanthrones, dibenzpyrene quinones, anthrimidocarbazols, naphthacridones, indigo, thioindigo, indirubin, etc., 20 including derivatives thereof, such as their halogen, nitro, sulfur, and/or alkoxy derivatives.

Examples of vat dyestuffs with which the present invention may be employed are such indigoid 25 and thioindigoid dyestuffs as the following:

|                                                                                |                      |
|--------------------------------------------------------------------------------|----------------------|
| National vat orange R.                                                         | Color Index No. 1217 |
| National vat red violet RH.                                                    | Color Index No. 1212 |
| 5,5'-dichlor-7,7'-dibrom indigo.                                               | Color Index No. 1188 |
| National brilliant indigo 4G.                                                  | Color Index No. 1189 |
| 30 National brilliant indigo B.                                                | Color Index No. 1190 |
| National brilliant indigo 4B.                                                  | Color Index No. 1184 |
| National vat scarlet G.                                                        | Color Index No. 1228 |
| National vat brown G (dinaphthyl-thioindigo)                                   |                      |
| National vat violet R.                                                         | Color Index No. 1222 |
| National vat green G.                                                          | Color Index No. 1199 |
| 35 National vat pink (6,6'-dichlor-4,4' dimethyl-2,2'-bis-thio-naphthenindigo) | Color Index No. 1210 |
| National vat pink BG.                                                          | Color Index No. 1196 |
| National vat yellow G.                                                         | Color Index No. 1170 |
| National vat yellow R.                                                         |                      |
| And such anthraquinone vat dyes as the following:                              |                      |
| National carbanthrene blue RS.                                                 | Color Index No. 1106 |
| National carbanthrene blue 3G.                                                 | Color Index No. 1109 |
| 40 National carbanthrene blue GCD.                                             | Color Index No. 1113 |
| National carbanthrene yellow G.                                                | Color Index No. 1118 |
| National carbanthrene golden orange 2RT.                                       | Color Index No. 1097 |
| National carbanthrene golden orange G.                                         | Color Index No. 1096 |
| National carbanthrene blue green FFB.                                          | Color Index No. 1173 |
| National carbanthrene violet 2R.                                               | Color Index No. 1104 |
| National carbanthrene dark blue DR.                                            | Color Index No. 1099 |
| National carbanthrene flavine GC.                                              | Color Index No. 1095 |
| 45 National carbanthrene red violet 2RNX.                                      | Color Index No. 1161 |
| National carbanthrene brilliant green supra.                                   | Color Index No. 1101 |
| National carbanthrene green B.                                                 | Color Index No. 1102 |
| National carbanthrene brown AR.                                                | Color Index No. 1151 |
| National carbanthrene olive R.                                                 | Color Index No. 1150 |
| National carbanthrene red BN.                                                  | Color Index No. 1162 |
| National carbanthrene red AFF.                                                 | Color Index No. 1133 |
| 50 National carbanthrene black J.                                              |                      |

Furthermore, mixtures of two or more vat dyes may be employed, for example when it is desired to produce compound shades such as scarlets, 55 navy blues, blacks and browns.

The invention is not restricted to any particular method of dyeing but includes the dyeing of piece goods and raw cotton stock (unspun cotton fiber) in a vat, the dyeing of piece goods (cotton, 60 ton, rayon, etc.) by padding in a reduced bath, machine dyeing of raw cotton stock, dyeing of yarn (cotton or rayon) on beams or in package dyeing machines, etc.

The alkyl salts of the present invention are 65 particularly valuable in the dyeing of so-called "gray-goods" (unbleached cotton fabrics, raw regenerated cellulose fabrics and the like) with vat dyes, inasmuch as the dyeings obtained with the aid of such alkyl ester salts have exceedingly high tinctorial value and excellent penetration 70 as compared with dyeing made in the absence of said alkyl ester salts.

The following examples, in which the parts are 75 by weight, will serve to illustrate the invention.

### Example 1

Mercerized cotton piece goods are dyed in a vat (jigger) as follows:—

12.75 pounds of National carbanthrene blue 5 GCD paste (containing about 17% of dye solids) are mixed with

8.16 pounds of sodium isobutyl sulfate, then 1 gallon cold water is added.

After dissolution of the sodium isobutyl sulfate 10 is complete the mixture is passed through a fine screen. A speckless paste of excellent quality is obtained, which is then added to the following composition contained in the jigger:

|                             |             |    |
|-----------------------------|-------------|----|
| Caustic soda.               | 10 pounds   | 15 |
| Sodium hydrosulfite (conc.) | 10 pounds   |    |
| Water.                      | 100 gallons |    |

The temperature is raised to 110° F. and after 20 complete reduction of the vat dye, dyeing is started at this temperature. After one passage of the goods through the bath an additional 5 pounds of sodium hydrosulfite (conc.) is added to the bath. The temperature of the bath is raised during 30 minutes to 125° F. The dyed cloth is 25 washed once with water, is then passed four times through a sodium perborate bath (containing 2 pounds of sodium perborate per 100 gallons) at a temperature of 120° F., is then washed twice with cold water, passed five times through a boiling 30 soap solution (containing 3 pounds of ordinary soap per 100 gallons), then rinsed, washed, dried and calendered.

The isobutyl sodium sulfate may be prepared, 35 for example, by reacting 516 parts of isobutyl alcohol with 813 parts of chlorsulfonic acid at a temperature of about 14° to 16° C.; adding the resulting reaction mixture slowly to 8100 parts of water to which 418 parts of hydrated lime, Ca(OH)<sub>2</sub>, have been added, while cooling the resulting mass to a temperature of about 20° C.; 40 filtering off calcium sulfate; converting the calcium isobutyl sulfate, contained in the filtrate, to sodium isobutyl sulfate, for example, by treating with sodium carbonate and removing calcium carbonate; and recovering the sodium isobutyl sulfate in the form of a dry solid. 45

### Example 2

100 parts of boiled off cotton yarn is dyed in a package dyeing machine with a dye liquor containing 50 the following ingredients:

|                                                                                                                                                        | Parts  |
|--------------------------------------------------------------------------------------------------------------------------------------------------------|--------|
| National carbanthrene blue DR paste (containing about 16% of dye solids) or National carbanthrene violet 2R paste (containing about 11% of dye solids) | 55     |
| Caustic soda.                                                                                                                                          | 5      |
| Sodium hydrosulfite.                                                                                                                                   | 2½     |
| Sodium isobutyl sulfate and sufficient water to give proper circulation and dyeing conditions (e. g., about 80 to 160 parts)                           | 3 to 4 |

The conditions of dyeing are the same as usual. After dyeing, the yarn is rinsed, oxidized with 65 2% sodium perborate solution, rinsed, soaped, rinsed and dried. The shades come out bright and very even.

It is obvious that in preparing the dye liquors of the above examples the ingredients may be incorporated in various ways. Further, the salt 70 of the acid alkyl ester may be added directly to the dye bath or may be preliminarily mixed with the vat dyestuff paste and the mixture added to the dye bath.

Instead of the isobutyl sodium sulfate em- 75

ployed in the above examples, any of the other alkyl ester salts herein described may be employed. For instance, in the above Example 2 the isobutyl sodium sulfate may advantageously be replaced by sodium isobutyl-boro-sulfate. (The sodium isobutyl boro-sulfate may be prepared, for example, by stirring 918 parts of 100% sulfuric acid with 200 parts of boron trioxide at a temperature of 75° C. until a uniform solution results; then adding 320 parts of isobutyl alcohol in a slow stream with agitation while keeping the temperature at 30 to 35° C.; after stirring this solution two hours running it into a mixture of 2000 parts of 40% caustic soda and 1000 parts of isobutyl alcohol while stirring and cooling; permitting the resulting mixture to stratify; drawing off the aqueous layer; neutralizing that remaining isobutyl alcohol layer with sodium carbonate or caustic soda, heating it to boiling and filtering hot; and drying the filtrate under vacuum on a rotary drum drier.)

The presence of the salts of the acid alkyl sulfates in the dye baths and liquors produces the following advantageous results:

(1) The dye baths are more completely exhausted;

(2) Owing to the advantageous levelling and penetrating action of the said alkyl ester salts, the depth of dyeing is better equalized, giving extremely even results and excellent penetration. This is particularly true for such dyes as National carbanthrene blue GCD, National carbanthrene violet 2R, National carbanthrene blue BCL, National carbanthrene dark blue DR, etc.;

(3) Due to the increased penetration there is better fixation of the dyestuff; and

(4) Due to more perfect dyeing conditions, the brilliancy of the dyeings is enhanced.

Similar improved results may be obtained by substituting 12.75 pounds of the vat dye powder described in Example 10 of copending application Serial No. 673,030 filed May 26, 1933 (which contains isobutyl sodium sulfate as a part thereof) for the vat dye paste and sodium isobutyl sulfate of Example 1, and by substituting 5 parts of the vat dye powders of Examples 3 and 4 of said copending application Serial No. 673,030 for the vat dye paste and sodium isobutyl sulfate of Example 2, the amount of water being correspondingly increased.

As above indicated, the advantageous action of the salts of the acid alkyl esters as assistants in the dyeing also may be secured by pretreating the fiber with the salt of the acid alkyl ester. The following example illustrates such pretreatment.

#### Example 3

Bleached or unbleached cotton cloth is padded with a solution containing, for example, about 5 to about 30 parts per 1000 parts of water of sodium isobutyl sulfate or any of the other salts of acid alkyl esters herein described, for example by passing the cloth through the solution contained in a padding box equipped with squeeze rolls. Preferably, the padding liquor also contains about 2 to about 5 parts of gum tragacanth or other suitable thickener per 1000 parts of liquor. The pressure of the squeeze rolls is preferably so regulated that the cloth retains its own weight of the padding liquor. The padded cloth is then passed through a hot air drier or over hot cans, is rolled up and is then ready for printing or dyeing. The penetration obtained this way is superior, especially for lighter shades. This

process is particularly suitable for artificial fibers of the regenerated cellulose type.

It will be understood that the dyeing process as herein described may be carried out with dye baths and dye liquors containing additional assistants such as one or more of the following hydrotropic substances, enolyzing substances, heavy metal compounds acting as reduction accelerators, catalysts or "boosters", etc.

This application is a continuation-in-part of 10 applications Serial Nos. 673,030 and 673,031, filed May 26, 1933.

I claim:

1. In the dyeing of textile fibers by forming a non-acid solution of leuco-compound of a vat dye and treating the fiber with said solution, the improvement which comprises carrying out the dyeing with the aid of a soluble salt of an acid alkyl ester containing not more than 5 carbon atoms in the alkyl group and derivable from a polybasic inorganic acid and an aliphatic alcohol containing not more than 5 carbon atoms.

2. In the dyeing of textile fibers of the vegetable type by forming an alkaline solution of a leuco-compound of a vat dye and treating the fiber with said solution, the improvement which comprises carrying out the dyeing in the presence of a soluble salt of an acid alkyl ester containing not more than 5 carbon atoms in the alkyl group and derivable from a polybasic inorganic acid and an aliphatic alcohol containing not more than 5 carbon atoms.

3. In the dyeing of textile fibers of the vegetable type by forming an alkaline solution of a leuco-compound of a vat dye and treating the fiber with said solution, the improvement which comprises carrying out the dyeing in the presence of a soluble salt of an acid alkyl ester having the formula  $(RO)_x-A-(OH)_{n-x}$  in which R represents an aliphatic hydrocarbon radical which contains not more than 5 carbon atoms, A represents the radical  $SO_2$  or the radical  $PO$ , n represents the number of replaceable hydrogen atoms in the uncombined polybasic acid from which the ester is derivable, and x represents a whole number not greater than 1.

4. In the dyeing of textile fibers of the vegetable type by forming an alkaline solution of a leuco-compound of a vat dye and treating the fiber with said solution, the improvement which comprises carrying out the dyeing in the presence of an alkali metal salt of an acid alkyl ester having the formula  $(RO)_x-A-(OH)_{n-x}$  in which R represents an aliphatic hydrocarbon radical which contains not more than 5 carbon atoms, A represents the radical  $SO_2$  or the radical  $PO$ , n represents the number of replaceable hydrogen atoms in the uncombined polybasic acid from which the ester is derivable, and x represents a whole number not greater than 1.

5. In the dyeing of textile fibers of the vegetable type by forming an alkaline solution of a leuco-compound of a vat dye and treating the fiber with said solution, the improvement which comprises carrying out the dyeing in the presence of an organic amine salt of an acid alkyl ester having the formula  $(RO)_x-A-(OH)_{n-x}$  in which R represents an aliphatic hydrocarbon radical which contains not more than 5 carbon atoms, A represents the radical  $SO_2$  or the radical  $PO$ , n represents the number of replaceable hydrogen atoms in the uncombined polybasic acid from which the ester is derivable, and x represents a whole number not greater than 1.

6. In the dyeing of textile fibers by forming a

non-acid solution of a leuco-compound of a vat dye and treating the fiber with said solution, the improvement which comprises incorporating an alkali metal salt of an acid alkyl sulfate containing not more than 5 carbon atoms in the alkyl group into a dye bath containing a non-acid solution of a leuco-compound of a vat dye, and working the fiber in the resulting bath.

7. In the dyeing of textile fibers of the vegetable type by treatment with a vat dye, the improvement which comprises incorporating an alkali metal salt of an acid alkyl sulfate containing 3 to 5 carbon atoms in the alkyl group into a dye bath containing an alkaline solution of a vat dye in the reduced form, and working the fiber in the resulting bath.

8. In the dyeing of textile fibers of the vegeta-

ble type by treatment with a vat dye, the improvement which comprises incorporating isobutyl sodium sulfate into a dye bath containing an alkaline solution of a vat dye in the reduced form, and working the fiber in the resulting bath.

9. In the dyeing of textile fibers of the vegetable type by treatment with an alkaline solution of a leuco-compound of a vat dye, the improvement which comprises treating the fiber to be dyed with a solution of a salt of an acid alkyl ester containing not more than 5 carbon atoms in the alkyl group and derivable from a polybasic inorganic acid and an aliphatic alcohol containing not more than 5 carbon atoms, and subjecting the treated fiber to the dyeing process.

5

10

15

JEAN G. KERN.